

# UNITED STATES PATENT OFFICE.

WILLIAM F. NOLAN, OF ST. PAUL, MINNESOTA.

## COPPER ALLOY.

1,074,285.

Specification of Letters Patent. Patented Sept. 30, 1913.

No Drawing.

Application filed April 19, 1912. Serial No. 691,978.

To all whom it may concern:

Be it known that I, WILLIAM F. NOLAN, a citizen of the United States, residing at St. Paul, in the county of Ramsey and State 5 of Minnesota, have invented a new and useful Copper Alloy, of which the following is a specification.

My invention relates to means and process for hardening copper and brass, and the 10 object of the invention is to enable articles made of copper or of brass, or of any alloy containing copper, to retain its form and finish of surface under considerable pressure, and to be more durable when exposed 15 to friction, as in journal boxes, and to perform service as cutting tools for wood and other material.

The invention involves an alloy which may be considerably varied without diverging 20 from the scope and spirit of the invention.

My composition consists of the following ingredients combined in the proportions stated, viz:

25 Copper ----- 98.15 per cent.  
Manganese ----- 1.48 per cent.  
Vanadium ----- 0.25 per cent.  
Aluminum ----- 0.12 per cent.

30 These ingredients are compounded and used as follows: Put the manganese, the vanadium and the aluminum in a crucible and apply heat until they commence to melt, then put in a small quantity of borax; as 35 soon as the borax is applied put in the copper; melt the mass until it flows freely, then

mix it by stirring, and pour it in molds. While yet dark red remove it from the mold and immerse it in oil; whale oil or lard oil is suitable. In this way the copper will be 40 about as hard as tool steel that has been fully hardened and then drawn to a blue color. If a greater or less hardness is desired, increase or decrease the other ingredients of the compound without changing the 45 quantity of the copper or brass to be hardened. If the article thus molded is to be drilled, turned, planed or filed, such work should be done before the article is immersed in the oil, and after the machine work is 50 done the article should be heated to a dark red color and immersed in the oil. From this description it will be understood that the brass or copper having said compound mixed into it may have its temper drawn 55 out by heat, and may be hardened at any time by heating it and immersing it in oil.

What I claim is:

1. An alloy consisting of copper, manganese, vanadium and aluminum. 60
2. An alloy consisting of copper, manganese, vanadium and aluminum in about the following proportions: copper 98.15 per cent., manganese 1.48 per cent., vanadium 0.25 per cent., aluminum 0.12 per cent. 65

In testimony whereof I affix my signature, in presence of two witnesses.

WILLIAM F. NOLAN.

Witnesses:

J. M. BEMANS,  
J. L. SMITH.